

# UNITED STATES PATENT OFFICE.

WILLIAM HENRY PERKIN, JR., OF MANCHESTER, ENGLAND, ASSIGNOR OF ONE-HALF TO WHIPP BROTHERS & TOD LIMITED, OF MANCHESTER, ENGLAND.

## FIREPROOFING TEXTILE MATERIAL.

No. 844,042.

Specification of Letters Patent.

Patented Feb. 12, 1907.

Application filed April 18, 1902. Serial No. 103,637. (Specimens.)

*To all whom it may concern:*

Be it known that I, WILLIAM HENRY PERKIN, Jr., Ph. D., F. R. S., a subject of the King of Great Britain and Ireland, residing at 5 Owen's College, in the city of Manchester, in the county of Lancaster, England, professor of organic chemistry, have invented certain new and useful Improvements in Fireproofing Goods, of which the following is a specification.

This invention relates to the treatment of raw cotton or cotton or other fibrous or textile goods (and especially flannelet) for rendering them less inflammable than hitherto by fixing an insoluble compound in the fibers of the material, so that they can be repeatedly washed and still retain their resistance to ignition.

My present invention consists in treating 20 the goods first with salt (such as sodium stannate) containing the oxid of a metal in its acid radical, then drying, then treating the said goods with a metallic salt not containing the oxid of a metal in its acid radical, but capable of forming an insoluble compound with the stannate, and then drying or drying and steaming the goods. An insoluble fireproofing compound is thus formed or deposited by precipitation directly in and upon the 25 fibers of the goods, so that it neither washes out when the material is subjected to domestic washings nor crumbles out in wear.

For the first bath I use a stannate, preferably sodium stannate. As examples of metallic salts which do not contain the oxid of a metal in their acid radicals, but which are capable of forming an insoluble compound with the deposit from the first bath, I mention soluble salts of zinc, aluminium, copper, and 30 nickel, such as acetate of zinc, acetate of aluminium, sulfate of copper, and sulfate of nickel.

The following is an example of the way in which the process may be carried out in practice according to this invention, (the parts given in the example are by volume.) The goods are treated with a solution of stann-

nate of soda of 16° Baumé and are then dried and then treated with a bath containing zinc-acetate solution of 17° Baumé, and 50 afterward the goods are dried or both dried and steamed. An insoluble body consisting partly of stannic acid and partly of a compound containing stannic acid is thus left in the fibers of the material after the second 55 treatment. By drying the first bath in the material after impragnation the stannate is brought within or in close contact with the fibers and does not wash away during the subsequent treatment. A portion of it becomes at the same time permanently fixed in the fibers as stannic acid, the remainder being afterward fixed (as an insoluble compound containing stannic acid) by the second bath.

I claim as my invention—

1. The process described of fireproofing fibrous and textile materials, said process consisting in preparing two separate baths, the first bath being a solution of a stannate, and the second bath being a solution of metallic salt free from the oxid of a metal in its acid radical, but capable of forming an insoluble compound with the stannate, saturating the goods first with the stannate-bath, then 70 drying the goods, and afterward saturating 75 the goods with the aforesaid second bath, and thereby forming an insoluble compound upon the goods to make them fireproof, and finally drying, for the purpose set forth.

2. The process described of fireproofing 80 fibrous and textile materials, said process consisting in first treating the same with a solution of a stannate, then drying, and then treating with a solution of an acetate capable of forming an insoluble compound with 85 the deposit from the first bath, and finally drying.

In testimony whereof I affix my signature in presence of two witnesses.

WILLIAM HENRY PERKIN, JUNIOR.

Witnesses:

WILLIAM GERALD REYNOLDS,  
PERCY READ GOLDRING.